

## UNITED STATES PATENT OFFICE.

GEORGES REYNAUD, OF PARIS, FRANCE.

## PROCESS OF MAKING ACHROO-DEXTRIN.

SPECIFICATION forming part of Letters Patent No. 761,542, dated May 31, 1904.

Application filed March 3, 1904. Serial No. 196,433. (No specimens.)

*To all whom it may concern:*

Be it known that I, GEORGES REYNAUD, engineer, of 5 Rue Salneuve, in the city of Paris, Republic of France, have invented Improvements Relating to the Manufacture of Achroo-Dextrin by the Treatment of Peat, of which the following is a full, clear, and exact description.

A process for the treatment of peat for the purpose of manufacturing industrially dextrin (achroo-dextrin) has been described in the application for Letters Patent of the United States, Serial No. 122,817, filed by me on September 10, 1902, and allowed on November 7, 1903, this process consisting in diluting the peat in twice its weight of water and in heating under pressure this dilution in an autoclave or digester at a temperature of 160° centigrade for about an hour and a half for the purpose of converting into achroo-dextrin the amylaceous matters of the peat.

Experience has shown that this temperature of 160° centigrade should not be exceeded and that this process of treatment should be applied exclusively to neutral peats.

This invention relates to a process for the treatment of acid peats, which are much more frequent.

This process consists, essentially, in diluting the peat in three to five times its weight of water and in heating this dilution in a digester under a low pressure at a temperature of 110° to 150° centigrade, according as the peat to be treated is more or less acid. The length of the operation may also be varied according to the degree of acidity of the peat. Under the influence of this temperature and of the humic acid which is contained in the peat the amylaceous matters of the latter begin to be converted after about twenty minutes of treatment in dextrin or, more exactly, achroo-dextrin. The operation is entirely finished in about one hour and even less, if the peat is very acid. The aqueous solution withdrawn from the digester may then be employed directly for the industrial exploitation of the achroo-

dextrin, or it may be submitted to a second operation for the purpose of converting it into alcohol.

This process permits of obtaining industrially, not erythrodextrin as the processes ordinarily employed for the manufacture of dextrin, but directly achroo-dextrin capable of advantageously replacing dextrin in its industrial applications by reason of its lower density.

This process does not necessitate the presence of any acid or other auxiliary substance. It is extremely economical. The manipulation is convenient and presents no danger. No special construction is requisite for the apparatus, which are not liable to injury and the maintenance of which is less costly. This process obviates, therefore, the defects inherent in the employment of acids.

In the application of my said process I may employ any kind of autoclave or digester apparatus—for example, a single apparatus or several appliances connected so as to form a battery—and any convenient method of heating may be adopted.

I claim—

The herein-described process for treating acid peats for the industrial manufacture of achroo-dextrin, consisting in mixing the peat to be treated in three to five times its weight of water and heating this mass under a low pressure in a digester, to a temperature of 110° to 150° centigrade during half an hour to an hour, according to the degree of acidity of the peat, for the purpose of converting the amylaceous matters of the peat into achroo-dextrin.

The foregoing specification of my improvements relating to the manufacture of achroo-dextrin by the treatment of peat signed by me this 17th day of February, 1904.

GEORGES REYNAUD.

Witnesses:

HANSON C. COXEY,  
RENÉ THIRIOT.